

# UNITED STATES PATENT OFFICE.

WARREN F. BLEECKER, OF PITTSBURGH, PENNSYLVANIA.

## METALLURGICAL PROCESS.

1,094,114.

No Drawing.

Specification of Letters Patent. Patented Apr. 21, 1914.

Application filed May 3, 1913. Serial No. 765,249.

To all whom it may concern:

Be it known that I, WARREN F. BLEECKER, of Pittsburgh, in the county of Allegheny and State of Pennsylvania, have invented 5 certain new and useful Improvements in Metallurgical Processes; and I do hereby declare the following to be a full, clear, and exact description of the invention, such as will enable others skilled in the art to which 10 it appertains to make and use the same.

This invention relates to improvements in processes for the production of alloys,—the object of the invention being to provide a simple and efficient process of making alloys, 15 such, for example, as ferro-vanadium, ferro-uranium and ferro-chromium, which shall be low in carbon, without resort to the use of such reducing agents as silicon, aluminum, ferro-manganese and the like which have a 20 deleterious effect upon the alloy.

A further object is to provide a process for making alloys, wherein the materials are reduced with carbon and still produce an alloy low in carbon.

25 With these objects in view, the invention consists in reducing a metallurgical mixture with excess of carbon to produce an alloy high in carbon and continuing the reduction process with slag forming material and 30 added unreduced metallurgical material to produce an alloy low in carbon.

The invention further consists in mixing metallic oxids and reducing the same with an excess of carbon to produce an alloy high 35 in carbon, and then continuing the reduction process with slag forming material and added unreduced oxids to produce an alloy low in carbon.

40 The invention further consists in certain novel steps in the process of making alloys low in carbon, as hereinafter set forth and pointed out in the claims.

In carrying my process into effect, I first 45 smelt metallic oxids or salts, such as ferric oxide and vanadium, uranium or chromium oxide, preferably in an electric furnace, with an excess of carbon and the necessary elements to form a fluid slag. The slag forming material to be used will depend upon 50 the impurities present in the oxids.

The alloy resulting from the above-described reducing step of the process will be an alloy high in carbon, a large proportion of which latter will be present as carbids.

A very large excess of carbon in this step of 55 the process is not necessary so long as enough shall be employed to effect complete reduction of all the metallic elements present in the material being reduced. The alloy, high in carbon, resulting from the first step 60 of the process will, preferably, be reduced to a suitable fineness and mixed with a calculated amount of unreduced oxids and slag forming material, and then subjected to a reducing temperature as before, so that the 65 carbon content of the alloy will be reduced by the oxids. That is to say, the carbon content of the alloy resulting from the first step of the process, is utilized for the reduction of further oxids and is replaced by the alloy 70 so reduced. The result is an alloy which is unusually low in carbon.

In smelting processes heretofore practised in making alloys, where a high carbon content such as would be obtained with one reduction, is not desirable, resort has been had to other reducing agents, such as silicon, 75 aluminum, ferro-manganese and the like, but these substances have a deleterious effect upon the alloy,—all of which is obviated in 80 the alloy produced by my improved method.

It is not absolutely essential to remove the alloy high in carbon, resulting from the first step of the process, from the furnace. Instead of doing this, slag may be drawn off, 85 and fresh oxids, together with slag forming material, added to the heated metal,—the important features of my invention comprising the complete reduction of the metal and the simultaneous production of slag 90 depleted in oxids, in the first step, and a second step consisting in the refining of the metal made in the first step, by removing the carbon with fresh oxids. Regarding slag forming material, the metallurgist will know 95 from an analysis of the raw materials what to add to make the slag. In some cases it may be a basic material, such as lime or magnesia, or it may be an acid material, such as alumina or silica.

Having fully described my invention what I claim as new and desire to secure by Letters-Patent, is:—

1. The herein described process, consisting in reducing a metallurgical mixture to 105 produce an alloy high in carbon, mixing with the reduced material a quantity of unreduced metallurgical material together with

slag forming material and heating the mixture whereby a portion of the carbon of the alloy is removed.

2. The herein described process, consisting in mixing with an alloy high in carbon, slag forming material and unreduced metallic oxide, and subjecting the whole to a reducing temperature.

3. The herein described process, consisting in reducing a mixture of metallic oxids with slag-forming material and an excess of carbon to produce an alloy high in carbon, and then mixing with such alloy slag forming material and unreduced oxids, and heating the same to produce an alloy low in carbon.

4. The herein described process, consisting in reducing pulverulent metallic oxide, slag forming material and an excess of carbon, to produce an alloy high in carbon, mix-

ing with such alloy slag forming material and unreduced metallic oxids, and heating the same to produce an alloy low in carbon.

5. The herein described process, consisting in reducing a mixture of ferric oxid and vanadium oxid with slag forming material and excess of carbon to produce an alloy high in carbon, then mixing with said alloy unreduced ferric and vanadium oxids and slag-forming material, and heating the same to produce a ferro - vanadium alloy low in carbon.

In testimony whereof, I have signed this specification in the presence of two subscribing witnesses.

WARREN F. BLEECKER.

Witnesses:

Jos. A. KELLY,  
Wm. GANLEY.